

## UNITED STATES PATENT OFFICE

ALAN R. LUKENS, OF WYOMING, OHIO, ASSIGNOR TO THE RICHARDSON COMPANY, OF LOCKLAND, OHIO, A CORPORATION OF OHIO

## DIELECTRIC SUBSTANCE

No Drawing.

Application filed April 12, 1923. Serial No. 631,743.

My invention relates to substances used for forming insulation, and more particularly for electrolyte containers, such as battery jars, one piece storage battery containers, and the like.

5 In forming the material of my invention, I proceed according to the so called Woodley process, which consists in mixing together with a bitumen, a wet or moistened filler of fibrous character, up to a stage when the filler is incorporated into the bitumen in a homogeneous manner, or in a state of substantially ultimate dispersion in the bitumen. Reference is hereby made to U. S. Patent to

10 Woodley No. 1,156,122, Oct. 12, 1915.

15 It is the object of my invention to provide a substance, which is moldable into various forms, and which has great tensile strength when cold, and a large elastic limit, and

20 which is not affected by the action of hot or cold acid, is non-porous, will not swell, has a very large resistance to low frequency electric currents, and is not affected when in the presence of electrolytic action.

25 Such a substance is fitted pre-eminently for molding into storage battery containers, into which compartments are formed to take the place of the present day individual rubber cell, the electrolyte and plates being set

30 directly into the said compartments.

In forming my new material, I use an asphalt which is a blend, preferably high in gilsonite, so as to give cohesiveness and adhesiveness, and I incorporate into this asphalt

35 a filler of mineral character, and a fibrous material, to give hardness, and tensile strength.

The exact nature of the asphalt or bitumen which is used, and the exact kind of mineral filler and of fibrous filler, may be varied to

40 suit different conditions, it being understood that in the following specification I am setting forth one particular example of my invention, giving preferred elements and treatment to gain the one special result in battery

45 containers, and that in the claims, which follow the specification, I desire to set forth the invention inherent in the subject matter set forth.

The mineral filler used by me has advantages which are two-fold, over any one of the

inert earths. In the first place it is acid resistant, and resists electrolytic action, which is not always the same thing. In the second place, it is of fibrous character, and acts as a reinforcing material.

55 The ordinary chrysotile asbestos of commerce, which appears in fibrous form, is not resistant to acid action, and hence cannot be employed. I find, however, that amphibole asbestos, which is acid proof, can be used with great advantage. The amphibole asbestos products of today are almost never in fibrous form, as when passed through the processes of segregating them from the rock in which they are found, the fibrous quality is almost entirely destroyed, due to inherent fragility. When removed by a water flotation process, this asbestos is left in an excellent fibrous form, which form, however, is more or less lost by any ordinary methods of drying.

60 In my process, however, it is of advantage to have the asbestos wet, when immersed into the bituminous bath.

65 I have found that a form of amphibole asbestos called actinolite, when removed by the water flotation process, familiar to mineralogists, and left in the wet stage, and merely pressed into a moist cake, forms the best mineral filler that I can use.

70 As to the ordinary fiber filler, I employ any organic or vegetable fibers, which I desire to have as long and tough as possible. The best fiber I have found to be a good clean cotton fiber.

75 I have discovered, however, that if I employ over about 14% of vegetable fiber, that the resulting product will not be acid resistant, or resistant to electrolytic action. By being acid resistant, I mean that the material formed up with a good bitumen, and the fiber intimately intermixed should not show marked discoloration in an acid bath, of 1.3 S. G. sulphuric acid at 125 degrees F. for 15 to 25 hours.

80 Particularly in battery containers, any tendency to show discoloration in the acid, results in a depositing action on the plates, whereby they are covered with the gummy products liberated from the bitumen. The usual rubber cell will show discoloration, de-

55

60

65

70

75

80

85

100

terioration and loss of shape, in case of over-charge by the service station or while in use, while the composition described herein shows no discoloration after many hours of over-charge.

5 As a safety factor, I prefer to use around ten percent of fiber, although the more fiber incorporated, the greater physical resistance is given to the composition. Cotton fibres 10 are the best which I have found because due to their length and strength, a smaller quantity by weight will produce better qualities, than larger quantities of other fibrous matter.

15 In one specific manufacturing method I place hot asphalt in a mixer, and add thoroughly wetted asbestos fiber of the character noted, and operate the mixing blades until the asbestos is thoroughly dispersed or distributed throughout the bituminous mass. I then continue the heat until the water disappears. I then add cotton fiber, with as little water as possible so long as each fiber is coated with the water, and continue the mixing 20 action in the presence of heat to maintain the bitumen in molten condition. The fiber of cotton may be incorporated first, and the asbestos last, if desired.

The asbestos material does not pulverize 30 when mixed in with the bitumen while wet, and does not act to grind up the vegetable fiber (cotton fiber). Also the degree of moisture, sufficient to merely film the surfaces of the fibers, speeds up the vibrating action, to 35 the degree that less time is necessary to eliminate the aqueous content from the final product. The mixing should be carried to the extent of colloidal relation.

A mixture of fibres in bitumen similar to 40 colloidal mixture results when the bitumen forms a complete coating on the fibres and a separating body between elementary fibres. This is accomplished by the Woodley patents of record in which the asphalt is imposed on 45 the fibres by agitation thereof in the presence of the asphalt when it is gummy enough to form the means of liberating the elementary fibres from each other, due to the working thereof. If the fibres are wet, this cools the 50 saturant, when it is of the type discussed in this specification, sufficiently to cause it to act in the manner noted.

The difference between a mixture of fibres similar to a colloidal mixture, and a mere 55 mixture of fibres and a binder, rests in the completeness of the external phase of the binder. A comparative test can be made up as follows which will indicate the result in a graphic way. First, saturate and coat a web 60 of fibres with a given per cent of soft asphalt. Second, liquify some more of the soft asphalt, and mix the fibres up in it, until as much uniformity as possible is gained, using the same proportions. Third, take half of the 65 mass of the second test and let it cool or add

some water, and proceed to mix further, so that the asphalt pulls like pulling candy and liberates the individual fibres. The result of the third process will have markedly different properties from the retained half of the second, and the second and third will have markedly different properties from the first.

70 The third step will present the feature of a colloidal mixture, and the term "fibration" has been coined to describe the process.

75 The product produced is increased in value by submitting the same to high pressures, and quickly sets under pressure into a very compact mass, entirely non-porous.

80 It is readily moldable, and in one process I form it up between male and female mold parts into a battery container with a plurality of integrally formed plate chambers or cells.

I also mold insulation pieces, for electrical equipment, which can be done quickly and cheaply, forming a product equal to phenolic condensation products, at least from the point of view of low frequency currents.

85 The percent of asbestos fiber will vary with the needs of the final product. In my battery container, I may use approximately equal parts asbestos fiber and bitumen, and the remainder vegetable fiber, although the proportions will vary depending upon the 90 bitumen used, and the purpose for which the product is intended. By the term "bitumen" in my claims is meant an organic or hydro-carbon binder of which asphalt is one.

95 Having thus described my invention, what I claim as new and desire to secure by letters 100 patent, is:—

1. A composition of matter for the purpose described, comprising bitumen, asbestos fibre in fibrous form, and of acid resistant character, and organic fibre, said organic fibre being less than substantially 15% of the mass, and said fibrous material being uniformly dispersed within the bitumen, and the individual fibres covered with the bitumen to an extent comparative to colloidal mixture.

105 2. A composition of matter for the purpose described comprising bitumen intermixed with acid resistant mineral matter in finely divided form, and organic fibre, said organic fibre being less than substantially 15% of the mass by weight, and said organic fibrous material being uniformly dispersed within the bitumen and the individual fibres covered with the bitumen and spaced from each other thereby to an extent comparative to colloidal mixture, and the whole mass molded under high pressure.

115 3. A molded article for use in the presence of electrolytic action comprising bitumen with finely divided acid resistant mineral matter and organic fibre, said organic fibre being in proportion of 10% to 15% of the mass by weight, and uniformly dispersed in the bitumen and coated thereby to an extent 120 comparative to colloidal mixture.

70

75

80

85

90

95

100

105

110

115

120

125

130

4. A moulded article for use in the presence  
of electrolytic action comprising bitumen  
with finely divided acid resistant mineral  
matter of fibrous nature and organic fiber,  
5 said organic fiber being less than substantially  
15% of the mass by weight, and uniformly  
dispersed in the bitumen and coated there-  
by to an extent comparative to colloidal mix-  
ture.

10

ALAN R. LUKENS.

15

20

25

30

35

40

45

50

55

60

65